

# UNITED STATES PATENT OFFICE.

VANCE P. EDWARDES, OF MADISON, WISCONSIN, ASSIGNOR TO THE UNITED STATES OF AMERICA.

## MANUFACTURE OF CELLULOSE.

1,310,694.

Specification of Letters Patent. Patented July 22, 1919.

No Drawing.

Application filed January 18, 1919. Serial No. 271,891.

*To all whom it may concern:*

Be it known that I, VANCE P. EDWARDES, a citizen of the United States, residing at Madison, in the county of Dane and State 5 of Wisconsin, have invented certain new and useful Improvements in the Manufacture of Cellulose, of which the following is a specification.

This invention relates to improvements in 10 the manufacture of cellulose from any material containing cellulose and has for its chief object the production of a finished, pure product more closely resembling pure cellulose in physical and chemical character- 15 istics than any heretofore produced.

One object of the invention is to provide a satisfactory process for obtaining from wood and vegetable growth a cellulose which can be satisfactorily substituted for 20 cotton in the manufacture of nitrocellulose, surgical dressings, and other commercial uses.

The process provides for the treatment of 25 wood pulp, which has been given a preliminary treatment by the sulfite process, with a secondary treatment with a weak solution of caustic soda. As a result of the treatment the pulp loses about 20% of surplus undesirable matter, the physical character- 30 istics have changed and it is much softer and more absorbent and the fiber length has not been shortened. The resultant pulp can be bleached with a much smaller proportion of bleaching chemical than could 35 the untreated material.

The process may be operated more effectively and at a much lower cost than any known process. The above and other advantageous features will be set forth in the 40 following detailed statement of the process. In commercial practice, sulfite pulping is carried on by two methods—the direct and indirect. In the first case, wood prepared in a suitable manner is charged into di- 45 gesters and a sufficient quantity of acid is run in. This acid is made up by bringing sulfur dioxide gas into contact with calcium or magnesium hydroxides, or a mixture of the two, or other suitable bases and water 50 in sufficient quantities. The acid composition may vary within wide limits and there are a number of standard methods of preparation in use. It may contain various percentages of such bases as calcium and mag- 55 nesium or any one base to the total exclu-

sion of the other. Satisfactory pulp may be made with acid strength varying from 3.4 per cent, total sulfur dioxide, 1.7 per cent. free and 1.7 per cent. combined to 7 per cent. total, 6 per cent. free and 1 per cent. combined.

The percentage of total  $\text{SO}_2$  is limited by mechanical conditions of the operation. For instance, it has been found that when working with an acid of that composition 65 or stronger, it is impossible to place the cover of the digester on as the evolution of gas caused by the contact of the acid with the heated lining of the digester is sufficient to generate enough pressure to blow 70 off the cover.

The temperatures, pressures, and methods of cooking may also vary, not only with the acid used but with the judgment of the operator. For the quick cook, steam is ad- 75 mitted into the digester and pressures of 60 to 90 lbs., with maximum temperatures from 125° C. to 165° C., are carried for 5 to 12 hours, with a total cooking time varying from 6 to 14 hours. When the cook is 80 completed, the pulp is discharged under pressure from the digester, usually into a blow pit where it is drained and washed.

The indirect cook is made much after the same manner, although, as the name implies, 85 no direct steam is used, the heat being supplied by steam coils in the digester. The wood, in general, is prepared in the same manner as for the direct cook although the chips are usually longer. In this process 90 it is quite common to rotate the digesters in order to secure better circulation. The acid used here is much weaker than the average practice in the direct cook and will analyze as low as 2.8 per cent. total  $\text{SO}_2$ , 1.8 per 95 cent. free and 1 per cent. combined. The time of cooking is in the neighborhood of 40 hours, the maximum pressure not more than 60 lbs. and the maximum temperature about 135° C. It is quite common to steam 100 the wood before admitting acid. Usually the pulp is not discharged under pressure as in the direct cook but the pressure is relieved, the liquor blown off and then the pulp discharged. There are also combina- 105 tions of these two processes, in which both direct and indirect steam is used. Variations in the process may be made according to the conditions surrounding the operation of the process in the mill.

For nitration work, chemical rather than physical qualifications are the desideratum. The most important of these is measured by the solubility of the material in a 10% solution of potassium hydroxid under definite conditions.

Unbleached sulfite pulp contains from 18-30% and bleached sulfite pulp contains 30-40%, of potassium hydroxid soluble matter which by the alkaline digestion may be reduced to almost any figure desired, depending upon the treatment employed. After treatment, the pulp is very readily bleached with the consumption of far less chemicals than the untreated pulp.

The practice in commercial sulfite pulping is to reduce the wood as thoroughly as possible, leaving very small percentages of undercooked material. In such a case the yield 20 is in the neighborhood of 43%.

This pulp loses 20% or more when given the secondary alkaline treatment, thus reducing the final yield in a like proportion, and the following modification to the process 25 has been successfully carried out:

Wood prepared for pulping in the usual manner is so treated as to give a uniformly raw cook. By that is meant that the pulping process is not wholly complete. The 30 yield in such a case will be 50% or over and consequently the final yield, after the caustic digestion, greater than if thoroughly cooked pulp had been used. The pulp is separated from the liquor and is now ready for the secondary alkaline treatment of the invention. The pulp is cooked in a closed vessel or digester with from 5 to 15 per cent. of its weight of caustic soda in solution, the strength of which may vary from  $\frac{1}{2}$  to 2 35 per cent. and the ratio of the weight of liquor to the pulp may vary from 6 to 1 and from 12 to 1. Various concentrations and volumes of sodium hydroxid solutions may be used. Good results with wood pulp are to be had by using a solution of 10% and about 40 10% concentration, that is, for every 100 grams of pulp, 10 grams of sodium hydroxid made up to 1000 c. c. were used. Pressures and temperatures to be used vary with the 45 quality and kind of the pulp used and the quality of the pulp desired. The pressure and temperature within the closed vessel may be controlled as desired. The process may be conducted at a pressure of 10 pounds 50 and with a temperature of about 115° C. A satisfactory operation of the process has been conducted with a pressure of 50 pounds and a temperature of about 148° C.

When operating with 50 pounds pressure 60 it has been found that the caustic is completely exhausted at the end of one hour and it is believed nothing further is to be gained by keeping the material in the digester beyond that time. Regardless of the strength 65 of the solution, care must be taken not to

make the treatment too drastic. In such a case appreciable quantities of cellulose will be dissolved by the caustic and excessive loss occur. By properly regulating the severity of the treatment, this loss can be reduced to a 70 minimum.

It is known that efforts have been made to use a subsequent treatment of caustic soda on a sulfite pulp. All such suggested processes now known are chemically wasteful, 75 using many times the amount of chemicals used in the present process, and are not practicable mechanically. Emphasis is directed to the low chemical consumption of this process, the fact that the sulfite pulp is 80 undercooked, and to the operation of the process under very considerable pressure, for a relatively short time.

Without any further treatment, paper made from pulp which has been treated in 85 the manner indicated in all of the foregoing is very soft and absorbent, is in a condition suitable for the manufacture of nitrocellulose, though possibly a slight bleaching treatment may be necessary, contains no fluff 90 and has other properties which point to its adaptability as a surgical dressing. In addition to the two uses mentioned, others will suggest themselves, particularly where soft, absorbent material can be used.

What I claim is:

1. The process of producing cellulose which comprises treating fibrous vegetable material with acid sulfite liquor, separating the fibrous material from the liquor, treating the fibrous material with a solution of caustic soda, and subjecting it to a pressure of at least ten pounds and to a temperature of at least 115° C.

2. The process of producing cellulose 105 which comprises treating fibrous vegetable material with acid sulfite liquor, separating the fibrous material from the liquor, treating the fibrous material with a solution of caustic soda of  $\frac{1}{2}$ -2 per cent. strength and 110 constituting 5-15 per cent. of the weight of the fibrous material, and subjecting the mixture of fibrous material and caustic material to a pressure of at least ten pounds and a temperature of at least 115° C.

3. The process of producing cellulose which comprises treating fibrous vegetable material with acid sulfite liquor, separating the fibrous material from the liquor, treating the fibrous material with a solution 120 of caustic soda, and subjecting it to a pressure of at least ten pounds and to a temperature of at least 115° C., said heat and pressure treatment being maintained for at least one hour.

4. The process of producing cellulose which comprises treating fibrous vegetable material with acid sulfite liquor, separating the fibrous material from the liquor, treating the fibrous material with a solution of caus- 130

tic soda of  $\frac{1}{2}$ -2 per cent. strength and constituting 5-15 per cent. of the weight of the fibrous material, and subjecting the mixture of fibrous material and caustic material to a pressure of at least ten pounds and a temperature of at least 115° C., said heat and pressure treatment being maintained for one hour.

5. The process of producing cellulose which comprises treating fibrous vegetable material with acid sulfite liquor, separating the fibrous material from the liquor, treating the fibrous material with a solution of caustic soda constituting 5-15 per cent. of the weight of the fibrous material and subjecting the mixture of fibrous material and caustic material to a pressure of at least ten pounds and a temperature of at least 115° C.

20 6. The process of producing cellulose which comprises treating fibrous vegetable material with acid sulfite liquor, separating the fibrous material from the liquor, treating the fibrous material with a solution of caustic soda and constituting 5-15 per cent. of the weight of the fibrous material, and subjecting the mixture of fibrous material and caustic material to a pressure of at least ten pounds and a temperature of at least 115° C., said heat and pressure treatment being maintained for one hour.

7. The process of producing cellulose which comprises treating fibrous vegetable material with acid sulfite liquor, separating the fibrous material from the liquor, treating the fibrous material with a solution of caustic soda, and subjecting it to a pressure of at least fifty pounds and to a temperature of at least 148° C.

40 8. The process of producing cellulose which comprises treating fibrous vegetable material with acid sulfite liquor, separating the fibrous material from the liquor, treating the fibrous material with a solution of caustic soda, and subjecting it to a pressure greater than atmospheric pressure and to a temperature of at least 115° C.

9. The process of producing cellulose which comprises treating fibrous vegetable material with acid sulfite liquor, separating the fibrous material from the liquor, treating the fibrous material with a solution of caustic alkali, and subjecting it to a pressure greater than atmospheric pressure and 55 to a temperature of at least 115° C.

10. The process of producing cellulose which comprises treating fibrous vegetable material with acid sulfite liquor and cooking the material so treated to an underdone condition, separating the fibrous material from the liquor, treating the fibrous material with a solution of caustic soda and subjecting it to a pressure of at least ten pounds and to a temperature of at least 65 115° C.

11. The process of producing cellulose which comprises treating fibrous vegetable material with acid sulfite liquor and cooking the material so treated to an underdone condition, separating the fibrous material from the liquor, treating the fibrous material with a solution of caustic soda of  $\frac{1}{2}$ -2 per cent. strength and constituting 5-15 per cent. of the weight of the fibrous material, and subjecting the mixture of fibrous material and caustic material to a pressure of at least ten pounds and a temperature of at least 115° C.

12. The process of producing cellulose which comprises treating fibrous vegetable material with acid sulfite liquor and cooking the material so treated to an underdone condition, separating the fibrous material from the liquor, treating the fibrous material with a solution of caustic soda, and subjecting it to a pressure of at least ten pounds and to a temperature of at least 115° C., said heat and pressure treatment being maintained for one hour.

13. The process of producing cellulose which comprises treating fibrous vegetable material with acid sulfite liquor, and cooking the material so treated to an underdone condition, separating the fibrous material from the liquor, treating the fibrous material with a solution of caustic soda of  $\frac{1}{2}$ -2 per cent. strength and constituting 5-15 per cent. of the weight of the fibrous material, and subjecting the mixture of fibrous material and caustic material to a pressure of at least ten pounds and a temperature of at least 115° C., said heat and pressure treatment being maintained for one hour.

14. The process of producing cellulose which comprises treating fibrous vegetable material with acid sulfite liquor, and cooking the material so treated to an underdone condition, separating the fibrous material from the liquor, treating the fibrous material with a solution of caustic soda constituting 5-15 per cent. of the weight of the fibrous material and subjecting the mixture of fibrous material and caustic material to a pressure of at least ten pounds and a temperature of at least 115° C.

15. The process of producing cellulose which comprises treating fibrous vegetable material with acid sulfite liquor, and cooking the material so treated to an underdone condition, separating the fibrous material from the liquor, treating the fibrous material with a solution of caustic soda and constituting 5-15 per cent. of the weight of the fibrous material, and subjecting the mixture of fibrous material and caustic material to a pressure of at least ten pounds and a temperature of at least 115° C., said heat and pressure treatment being maintained for one hour.

16. The process of producing cellulose which comprises treating fibrous vegetable

material with acid sulfite liquor, and cooking the material so treated to an underdone condition, separating the fibrous material from the liquor, treating the fibrous material 5 with a solution of caustic soda, and subjecting it to a pressure of at least fifty pounds and to a temperature of at least 148° C.

17. The process of producing cellulose which comprises treating fibrous vegetable 10 material with acid sulfite liquor, and cooking the material so treated to an underdone condition, separating the fibrous material from the liquor, treating the fibrous material with a solution of caustic soda, and subjecting it 15 to a pressure greater than atmospheric pressure and to a temperature of at least 115° C.

18. The process of producing cellulose which comprises treating fibrous vegetable 20 material with acid sulfite liquor, and cooking the material so treated to an underdone condition, separating the fibrous material from the liquor, treating the fibrous material with a solution of caustic alkali, and subjecting it to a pressure greater than

atmospheric pressure and to a temperature 25 of at least 115° C.

19. The process of producing cellulose which comprises treating fibrous vegetable material with acid sulfite liquor, cooking the material stopping the cooking action before 30 the pulping action is complete, separating the fibrous material from the liquor, treating the fibrous material with a solution of caustic soda, and subjecting it to a pressure of at least ten pounds and to a temperature of at 35 least 115° C.

20. The process of producing cellulose which comprises treating fibrous vegetable material, with acid sulfite liquor, separating the fibrous material from the liquor, treating the fibrous material with a solution of caustic soda, and subjecting it to a pressure of at least fifty pounds and to a temperature of at least 148° C., said heat and pressure treatment being maintained for approximately one hour.

In testimony whereof I affix my signature.  
VANCE P. EDWARDES.